



US006136910A

**United States Patent** [19]**Virnelson et al.****Patent Number:** **6,136,910****Date of Patent:** **\*Oct. 24, 2000**[54] **DESICCANT MATRIX FOR AN INSULATING GLASS UNIT**[75] Inventors: **Bruce Virnelson, Valencia; Jin Song, Stevenson Ranch, both of Calif.**[73] Assignee: **PRC-Desoto International, Inc., Burbank, Calif.**

[ \* ] Notice: This patent issued on a continued prosecution application filed under 37 CFR 1.53(d), and is subject to the twenty year patent term provisions of 35 U.S.C. 154(a)(2).

[21] Appl. No.: **08/704,249**[22] Filed: **Aug. 28, 1996****Related U.S. Application Data**

[62] Division of application No. 08/444,964, May 19, 1995.

[51] **Int. Cl.<sup>7</sup>** ..... **C08K 3/34**[52] **U.S. Cl.** ..... **524/450; 524/296; 524/261; 524/265; 524/198; 524/199; 524/200; 427/210; 156/275.5**[58] **Field of Search** ..... 524/296, 450, 524/261, 245, 198, 199, 200; 156/275.5; 427/210[56] **References Cited****U.S. PATENT DOCUMENTS**

|           |         |                        |           |
|-----------|---------|------------------------|-----------|
| 3,758,996 | 9/1973  | Bowser .               |           |
| 3,791,910 | 2/1974  | Bowser .....           | 428/34    |
| 3,919,023 | 11/1975 | Bowser et al. ....     | 156/107   |
| 4,032,500 | 6/1977  | Koch et al. ....       | 152/504   |
| 4,042,736 | 8/1977  | Flint .....            | 428/34    |
| 4,120,999 | 10/1978 | Chenel et al. ....     | 428/34    |
| 4,153,594 | 5/1979  | Wilson, Jr. ....       | 524/59    |
| 4,215,164 | 7/1980  | Bowser .....           | 428/34    |
| 4,425,389 | 1/1984  | Schöllhorn et al. .... | 428/34    |
| 4,431,691 | 2/1984  | Greenlee .....         | 428/34    |
| 4,476,169 | 10/1984 | Nishino et al. ....    | 428/34    |
| 4,530,195 | 7/1985  | Leopold .....          | 52/717.02 |
| 4,587,289 | 5/1986  | Comert et al. ....     | 524/505   |
| 4,622,249 | 11/1986 | Bowser .....           | 428/34    |

|           |         |                             |            |
|-----------|---------|-----------------------------|------------|
| 4,669,241 | 6/1987  | Kelly .....                 | 52/204,597 |
| 4,775,719 | 10/1988 | Markevka et al. ....        | 525/125    |
| 4,808,255 | 2/1989  | Markevka et al. ....        | 156/307.3  |
| 4,820,368 | 4/1989  | Markevka et al. ....        | 156/307.3  |
| 4,835,130 | 5/1989  | Box .....                   | 502/62     |
| 4,891,269 | 1/1990  | Markevka et al. ....        | 428/423.1  |
| 4,950,344 | 8/1990  | Glover et al. ....          | 156/109    |
| 4,965,117 | 10/1990 | Lautenschlaeger et al. .... | 428/182    |
| 4,985,535 | 1/1991  | Takada et al. ....          | 528/272    |
| 4,994,309 | 2/1991  | Reichert et al. ....        | 428/34     |
| 5,017,653 | 5/1991  | Johnston .....              | 525/89     |
| 5,019,638 | 5/1991  | Müller et al. ....          | 528/83     |
| 5,061,749 | 10/1991 | Ito et al. ....             | 524/850    |
| 5,075,407 | 12/1991 | Cody et al. ....            | 528/71     |
| 5,091,444 | 2/1992  | Bauer et al. ....           | 523/209    |
| 5,106,663 | 4/1992  | Box .....                   | 428/34     |
| 5,120,379 | 6/1992  | Noda et al. ....            | 156/107    |
| 5,177,916 | 1/1993  | Misera et al. ....          | 52/172     |
| 5,189,096 | 2/1993  | Boutillier et al. ....      | 525/56     |
| 5,234,730 | 8/1993  | Lautenschlaeger et al. .... | 428/34     |
| 5,286,787 | 2/1994  | Podola et al. ....          | 524/773    |
| 5,304,623 | 4/1994  | Ito et al. ....             | 528/28     |
| 5,324,778 | 6/1994  | Boutillier et al. ....      | 525/56     |
| 5,340,887 | 8/1994  | Vincent et al. ....         | 525/477    |
| 5,342,873 | 8/1994  | Merz et al. ....            | 524/425    |
| 5,385,986 | 1/1995  | Frihart et al. ....         | 525/420.5  |
| 5,424,111 | 6/1995  | Farbstein .....             | 428/137    |
| 5,494,957 | 2/1996  | Moore et al. ....           | 524/504    |
| 5,641,575 | 6/1997  | Farbstein .....             | 428/423.1  |
| 5,849,832 | 12/1998 | Virnelson et al. ....       | 524/512    |

**FOREIGN PATENT DOCUMENTS**

1181519 2/1970 United Kingdom .

*Primary Examiner*—Blaine Copenheaver*Assistant Examiner*—John J. Guarriello*Attorney, Agent, or Firm*—Gifford, Krass, Groh, Sprinkle, Anderson & Citkowski, P.C.[57] **ABSTRACT**

This invention relates generally to spacer assemblies for insulating glass units. More specifically, this invention relates to a single component desiccant matrix which can be applied to the interior of a spacer assembly at room temperature. Upon exposure to the ambient atmosphere, the desiccant matrix irreversibly cures.

**32 Claims, 1 Drawing Sheet**



Fig-1



Fig-2

## DESICCANT MATRIX FOR AN INSULATING GLASS UNIT

This is a divisional of copending application Ser. No. 08/444,964 filed on May 19, 1995, pending.

### BACKGROUND OF THE INVENTION

#### I. Field of the Invention

This invention relates generally to methods and compositions for constructing insulating glass units and in particular, methods and compositions for making a desiccant matrix which is applied to a metal spacer assembly used in the construction of insulating glass units. Most specifically, the present invention relates to a powdered desiccant which is suspended in an atmospheric curing resin, the resin being in a liquid phase at room temperature.

#### II. Description of the Prior Art

Insulating glass units generally comprise a pair of glass sheets maintained in a spaced apart relationship to each other by a spacing and sealing assembly which extends around the periphery of the inner, facing surfaces of the glass sheets, to define a sealed and insulating air space between the glass sheets. A spacer assembly generally comprises an inner spacer-dehydrator element which extends around the periphery of the inside facing surfaces of the glass sheets. The inner surfaces of the glass sheets are attached to the outer surface of the spacer assembly by means of a sealant or adhesive.

In one typical form of insulating glass unit, the inner spacer-dehydrator element comprises a hollow metal spacer element generally adhered to the periphery of the inside, facing surfaces of the sheets, to provide an insulating air space. The metal spacer element is generally tubular in shape and filled with a desiccant material, which is put in communication with the insulating air space to absorb moisture therefrom, and to enhance the performance and durability of the unit. The desiccant prevents moisture condensation on the inner surfaces of the window panes.

There are several known ways of filling the spacer assembly with the desiccant material. One known way is to manually pour beads which serve as carriers for the desiccant in the spacer assembly. This method is unsatisfactory because it is both inefficient and labor intensive. Another approach to applying the desiccant material to the spacer assembly is to utilize a powdered molecular desiccant which is carried in a hot melt butyl thermoplastic carrier. There are numerous problems with this approach. Because the hot melt carrier must be maintained at an elevated temperature while the desiccant material is being applied to the spacer, this procedure requires elevated temperature application equipment, thereby increasing initial capital costs and operating costs. Additionally, since the desiccant impregnated spacers often times must be handled right after application of the desiccant material, the hot melt systems increase the likelihood that operators of the equipment as well as handlers of the spacers will get burned. Finally, the use of thermoplastic materials to carry the powdered desiccant may compromise the aesthetic integrity of the insulating glass unit in that even after installation, the desiccant carrier can remelt and/or sag if the window unit is exposed to elevated temperatures. This makes the use of thermoplastics as desiccant carriers highly undesirable for window units installed in locations having hot climates.

U.S. Pat. No. 4,622,249 discloses a silicone glazing adhesive/sealant as a desiccant carrier. The carrier material is a flexible, organic, room temperature vulcanizable adhe-

sive sealant material comprised of two components. One of the components comprises a base material and the other component comprises a curing agent or accelerator. Neither of the components is individually curable or vulcanizable. 5 When the two components are combined, a chemical cross linking reaction takes place which begins curing or vulcanizing the two-component material at room temperature.

U.S. Pat. No. 3,758,996 discloses a desiccant material which is carried in a thermoplastic carrier. In one example, the desiccant matrix is applied to the spacer assembly at a temperature above 250° F.

The present invention overcomes all of the problems of the prior art in that it provides a desiccant matrix for use in a spacer assembly of an insulating glass unit which can be applied as a single component and at room temperature. 10 Upon exposure to the atmosphere, the desiccant matrix irreversibly cures into a solid structure, thereby preventing the desiccant from running or sagging at some later date after installation of the window unit. Since the desiccant matrix can be applied as a single component and at room temperature, operating costs are kept down, as well as minimizing the potential risk of injury to workers who must handle the spacer assemblies. These and other advantages of 15 the present invention will be readily apparent from the description, the discussion and examples which follow.

### SUMMARY OF THE INVENTION

There is disclosed herein a spacer assembly for use in a 30 multiple pane window assembly comprising a powdered molecular sieve desiccant suspended in an atmospheric curing resin which is a liquid at room temperature. The composition of the desiccant matrix comprises, by weight, approximately 30 to 80% of a powdered molecular sieve desiccant, together with approximately 5 to 40% of an atmospheric curing resin.

In particular embodiments, the powdered molecular sieve desiccant has a pore size ranging from three angstroms to ten 35 angstroms. The desiccant may comprise a mixture of different pore-sized material. One particularly preferred molecular sieve desiccant comprises a blend of 97% 3A and 3% 13X desiccants. The liquid carrier is preferably an atmospheric curing resin which exists in a liquid state at room temperature. One particularly preferred group of atmospheric curing resins comprises alkoxy silane terminated polyurethanes. Another preferred group of resins comprises alkoxy silane terminated polyethers. Finally, a third group of 40 preferred resins comprises polydimethylsiloxanes. The composition may also include ancillary ingredients such as plasticizers, catalysts, and fillers. Some preferred plasticizers include phthalate esters, chlorinated paraffins, mineral oils, and silicon oils. The catalysts may include organotin compounds such as dibutyl tin dilaurate and dibutyl tin diacetate, as well as aliphatic titanates and amines. Small 45 volume fillers may include colorants, rheological materials and/or pigments.

### BRIEF DESCRIPTION OF THE DRAWINGS

FIG. 1 is a perspective view of a spacer assembly;

FIG. 2 is a cross-sectional view of a spacer assembly in 50 an insulating glass unit.

### DETAILED DESCRIPTION OF THE INVENTION

Referring to FIGS. 1 and 2, the present invention is directed to a spacer assembly 10 for use in a multiple pane

window unit, the interior of the spacer assembly **10** being filled with a desiccant matrix **12**. The desiccant matrix **12** can be applied to the spacer **14** at room temperature, and upon exposure to moisture and/or oxygen is irreversibly cured.

In the broadest sense, the present invention includes a powdered molecular sieve desiccant which is dispersed in an atmospheric curing resin which exists as a liquid at room temperature. Within the context of this disclosure, atmospheric "curing resins" are meant to include monomeric and low molecular weight polymeric materials which cross-link and/or polymerize upon exposure to a component of the ambient atmosphere, typically oxygen or water vapor.

Preferably, the powdered molecular sieve desiccant is present in the desiccant matrix **12** in a concentration of 30 to 80% by weight, more preferably 40-70% by weight, and most preferably 60% by weight. The liquid carrier is typically present in the desiccant matrix **12** in a range of 5 to 40% by weight, more preferably 10-25% by weight, and most preferably 22.2% by weight. The carrier further comprises atmospheric curing resins which exist in a liquid phase at room temperature. The desiccant matrix **12** may also include a catalyst, a plasticizer, as well as small volume fillers.

The powdered molecular sieve desiccant is preferably one which has a pore size ranging from three to ten angstroms, and mixtures thereof. It may further comprise synthetic zeolite, sodium aluminum silicate, or potassium aluminum silicate. Among some of the more preferred desiccants are powdered molecular sieve 3A and powdered molecular sieve 13X, as are known in the art. One particularly preferred desiccant comprises a blend of 97% 3A and 3% 13X desiccants.

The carrier for the desiccant is an atmospheric curing resin which exists in the liquid phase at room temperature. A preferable group of carriers for the desiccant comprises moisture cure polyurethanes, moisture cure polysulfides, polydimethylsiloxanes, and oxygen cure polysulfides. Some specific carriers include alkoxy acetoxy oxyamino silane terminated polyethers and polyether urethanes; alkyl siloxane polymers crosslinked with alkoxy acetoxy oxyamino organo functional silanes; moisture curable isocyanate functional poly oxyalkaline polymers and polyalkaline polymers; thiol functional polymers and oligomers (such as polyethers, polyether urethanes, polysulfides, polythioethers), suitably catalyzed to produce moisture curable systems; epoxide functional polymers and oligomers with moisture deblockable crosslinkers; and acrylic function polymers with deblockable crosslinkers. Most preferably, the carrier comprises alkoxy silane terminated polyurethanes, alkoxy silane terminated polyethers, or polydimethylsiloxane polymers. In one preferred formulation, the carrier comprises KANEKA MS, manufactured by KaneKagafuchi Chemical Company of Japan and distributed by Union Carbide. In a most preferred formulation, the carrier comprises PERMAPOL MS, manufactured by Courtaulds Coatings, Inc.

The specific organic catalyst used in the present invention will depend upon the particular carrier which is used. Preferable catalysts comprise organotin compounds, aliphatic titanates (having from one to twelve carbon atoms) such as lower alkyl titanates, and amines. Most preferably the catalyst comprises dibutyl tin dilaurate, dibutyl tin diacetate, tetrabutyl titanate, and tetraethyl titanate.

The selection of the plasticizer is also dependent upon the nature of the liquid resin. The most preferable plasticizers are phthalate esters, chlorinated paraffins, mineral oils, and

silicone oils. The selection of the plasticizer depends upon compatibility with the liquid resin, low cost, as well as having low volatility and low vapor pressure. A plasticizer having high volatility or high vapor pressure would be undesirable because it would fog the interior of the insulating glass unit. In a preferred formulation, the plasticizer comprises 0-30% by weight of the desiccant matrix **12**, more preferably 5-20% by weight, and most preferably 13.4% by weight.

Although the material will still cure without the addition of the catalyst, the addition of a catalyst provides for very rapid skin times, as well as faster curing times, which may be necessary in certain situations. It may also be desirable, in some instances, to add small amounts of fillers, colorants, pigments, rheological agents and the like.

The desiccant matrix **12** of the present invention may be prepared in the following manner. Preferably, the plasticizer is first disposed in a mixing vessel. In one preferred embodiment, the mixing vessel comprises a variable speed, multishaft unit, having a low speed sweep blade, a high speed disperser, and a low speed auger. The mixing vessel further comprises a 300 gallon, triple shaft vacuum mixer with cooling capabilities. The liquid polymer is then added to the plasticizer and mixing begins at low speed. Thereafter, the powdered molecular sieve desiccant is added to the mixture and the high speed disperser is activated to decrease the average particle size of the mixture as well as to increase uniformity within the mixture. At the point the desiccant is added, the mixing is conducted under vacuum so as to eliminate any exposure of the mixture to moisture. The fillers, colorants and the like, as well as the catalyst, are added last. The material is maintained under essentially dry conditions until such time as it is ready to be applied to the spacer assembly **10**.

The desiccant matrix **12** is applied to the interior of the spacer assembly **10** at room temperature. The application can be made by any conventional dispensing technique such as extruding, pumping, or the like. Upon exposure to the atmosphere, the desiccant matrix **12** irreversibly cures. Upon installation, the spacer assembly **10** is disposed between a plurality of glass sheets **16**. The spacer assembly **10** is adhered to the glass sheets **16** by means of a conventional sealant **18**, as is known in the art. The final curing of the desiccant matrix **12** generally takes place once the entire insulating glass unit **20** is installed.

The present invention will best be illustrated by the following series of examples:

#### EXAMPLE 1

All weights are in pounds, unless otherwise indicated.

- Step 1. Material: Phthalate ester plasticizer; Charge Weight: 762.5; % Weight: 22.66; Procedure: Charge. Mix under full vacuum at low speed for 10 minutes.
- Step 2. Material: PERMAPOL MS polymer 1; Charge Weight: 225; % Weight: 6.7; Procedure: Charge.
- Step 3. Material: PERMAPOL MS polymer 2; Charge Weight: 225; % Weight: 6.7; Procedure: Charge. Turn on cooling water.
- Step 4. Material: Organic treated clay; Charge Weight: 41; % Weight: 1.2; Procedure: Charge.
- Step 5. Material: Carbon black; Charge Weight: 20; % Weight: 0.6; Procedure: Charge. Mix at low speed for 5 minutes.
- Step 6. Material: Titanium dioxide; Charge Weight: 4086 gms; % Weight: 0.3; Procedure: Charge.
- Step 7. Material: Powdered molecular sieve 13X; Charge Weight: 155; % Weight: 4.6; Procedure: Charge.
- Step 8. Material: Ground calcium carbonate; Charge Weight: 45; % Weight: 1.34; Procedure: Charge. Turn on vacuum.

## 5

Mix with low speed blades at low setting and disperser at medium speed for 5 minutes.

Step 9. Material: Powdered molecular sieve 3A; Charge Weight: 1850; % Weight: 55; Procedure: Charge. Turn on vacuum, then close vacuum. Mix at low speed all blades for 5 minutes.

Step 10. Material: Fumed silica; Charge Weight: 15; % Weight: 0.4; Procedure: Charge. Turn on vacuum. Then close vacuum. Mix at medium speed all blades for 10 minutes.

Step 11. Material: Dibutyl tin dilaurate; Charge Weight: 715 g; % Weight: 0.05; Procedure: Charge.

## EXAMPLE 2

All weights are in pounds, unless otherwise indicated.

Step 1. Material: Phthalate ester plasticizer; Charge Weight: 762.5% Weight: 22.66; Procedure: Charge. Mix under full vacuum at low speed for 10 minutes.

Step 2. Material: PERMAPOL MS polymer 1; Charge Weight 225; % Weight: 6.7; Procedure: Charge.

Step 3. Material: PERMAPOL MS polymer 2; Charge Weight: 225; % Weight: 6.7; Procedure: Charge. Turn on cooling water.

Step 4. Material: Organic treated clay; Charge Weight: 41; % Weight: 1.2; Procedure: Charge.

Step 5. Material: Carbon Black; Charge Weight: 3065 g; % Weight: 0.2; Procedure: Charge. Mix at low speed for 5 minutes.

Step 6. Material: Powdered molecular sieve 13X; Charge Weight: 155; % Weight: 4.6; Procedure: Charge.

Step 7. Material: Ground calcium carbonate; Charge Weight: 45; % Weight: 1.34; Procedure: Charge. Turn on vacuum. Mix with low speed blades at low setting and disperser at medium speed for 5 minutes.

Step 8. Material: Powdered molecular sieve 3A; Charge Weight: 1850; % Weight: 55; Procedure: Charge. Turn on vacuum, then close vacuum. Mix at low speed all blades for 5 minutes.

Step 9. Material: Fumed silica; Charge Weight: 15; % Weight: 0.4; Procedure: Charge. Turn on vacuum. Then close vacuum. Mix at medium speed all blades for 10 minutes.

Step 10. Material: Dibutyl tin dilaurate, Charge Weight: 715 g; % Weight: 0.05; Procedure: Charge.

## EXAMPLE 3

The same protocol was used as set forth in Examples 1 and 2.

| Material                     | Weight (grams) | % Weight |
|------------------------------|----------------|----------|
| Phthalate ester plasticizer  | 162.51         | 22.0%    |
| KANEKA 20A                   | 100            | 13.6%    |
| Organic treated clay         | 10             | 1.4%     |
| Carbon black                 | 0.01           | 0.001%   |
| Titanium dioxide             | 2.0            | 0.3%     |
| Powdered molecular sieve 13X | 34.6           | 4.7%     |
| Ground calcium carbonate     | 17.9           | 2.4%     |
| Powdered molecular sieve 3A  | 409            | 55.3%    |
| Fumed silica                 | 3.4            | 0.5%     |
| Dibutyl tin dilaurate        | 0.5            | 0.1%     |
|                              | 740.02         | 100%     |

## 6

## EXAMPLE 4

The same protocol was used as set forth in Examples 1 and 2.

| Material                                  | Weight (grams) | % Weight |
|-------------------------------------------|----------------|----------|
| 18000 Centistoke silicone polymer         | 50             | 20.8%    |
| 50 Centistoke non-reactive silicone fluid | 52.0           | 21.6%    |
| Powdered molecular sieve 3A               | 125            | 51.9%    |
| Dibutyl tin dilaurate                     | 0.5            | 0.2%     |
| Powdered molecular sieve 13X              | 13.0           | 5.4%     |
| Carbon black                              | 0.2            | 0.08%    |
|                                           | 240.7          | 99.98%   |

The foregoing discussion and examples are merely meant to illustrate particular embodiments of the invention, and are not meant to be limitations on the practice thereof. It is the following claims, including all equivalents, which define the scope of the invention.

What is claimed is:

1. A desiccant matrix comprising: a powdered inorganic molecular sieve desiccant; and a carrier for said powdered inorganic molecular sieve desiccant, said carrier comprising an atmospheric curing resin which irreversibly partially crosslinks upon exposure to a component of an ambient atmosphere selected from the group consisting of oxygen and moisture, with complete crosslinking occurring thereafter.
2. The desiccant matrix of claim 1, wherein said powdered molecular sieve desiccant comprises a desiccant selected from the group consisting of synthetic zeolite, sodium aluminum silicate, and potassium aluminum silicate.
3. The desiccant matrix of claim 1, wherein said powdered molecular sieve desiccant comprises a mixture of 3A and 13X desiccants.
4. The desiccant matrix of claim 1, wherein said atmospheric curing resin comprises a moisture curing urethane.
5. The desiccant matrix of claim 4, wherein said moisture curing urethane comprises an alkoxy silane terminated polyurethane.
6. The desiccant matrix of claim 1, wherein said atmospheric curing resin comprises a moisture curing polysulfide.
7. The desiccant matrix of claim 1, wherein said atmospheric curing resin comprises an alkoxy silane terminated polyether.
8. The desiccant matrix of claim 1, wherein said atmospheric curing resin comprises a polydimethylsiloxane resin.
9. The desiccant matrix of claim 1, wherein said atmospheric curing resin comprises an oxygen curing polysulfide.
10. The desiccant matrix of claim 1, wherein said desiccant matrix further comprises a plasticizer.
11. The desiccant matrix of claim 10, wherein said plasticizer comprises a low volatility, low vapor pressure plasticizer selected from the group consisting of phthalate esters, chlorinated paraffins, silicon oils, and mineral oils.
12. The desiccant matrix of claim 1 wherein said powdered molecular sieve desiccant is present from 30 to 80 weight percent.
13. The desiccant matrix of claim 1 wherein said powdered molecular sieve desiccant is present from 55 to 65 weight percent.
14. The desiccant matrix of claim 1 wherein said atmospheric curing resin is present from 5 to 40 matrix weight percent.

**15.** The desiccant matrix of claim 1 wherein said atmospheric curing resin is present from 20 to 25 matrix weight percent.

**16.** A method of making a desiccant matrix comprising the steps of:

- providing a mixing vessel;
- excluding oxygen and moisture from said vessel;
- disposing a plasticizer in said vessel;
- disposing an atmospheric curing resin in said vessel, said resin being a liquid at room temperature and irreversibly crosslinking upon exposure to a component of an ambient atmosphere selected from the group consisting of oxygen and moisture; and
- disposing a powdered inorganic molecular sieve material in said vessel.

**17.** The method of claim 16 further comprising disposing a catalyst in said vessel.

**18.** The method of claim 17, wherein said catalyst comprises an organotin compound.

**19.** The method of claim 17, wherein said catalyst comprises a lower alkyl titanate.

**20.** The method of claim 17, wherein said catalyst comprises a compound selected from the group consisting of dibutyl tin dilaurate, dibutyl tin diacetate, tetrabutyl titanate, and tetraethyl titanate.

**21.** The method of claim 16, further comprising mixing said plasticizer, said resin, and said molecular sieve desiccant in said vessel while continuing to exclude oxygen and moisture therefrom.

**22.** A desiccant matrix consisting of:

30 to 80 matrix weight percent of a powdered molecular sieve desiccant in a carrier for said powdered molecular sieve desiccant, said carrier comprising an atmospheric curing resin which irreversibly partially crosslinks upon exposure to a component of an ambient atmosphere selected from the group consisting of oxygen and moisture, wherein said resin fully cures thereafter.

**23.** The desiccant matrix of claim 22 wherein said powdered molecular sieve desiccant is present from 40 to 70 weight percent.

**24.** The desiccant matrix of claim 22 wherein said powdered molecular sieve desiccant is present from 55 to 65 weight percent.

**25.** A desiccant matrix consisting essentially of:

30 to 80 matrix weight percent of a powdered molecular sieve desiccant in a carrier for said powdered molecular sieve desiccant, said carrier comprising an atmospheric curing resin which irreversibly partially crosslinks upon exposure to a component of an ambient atmo-

30

35

40

45

45

sphere selected from the group consisting of oxygen and moisture, wherein said resin fully cures thereafter.

**26.** The desiccant matrix of claim 25 wherein said catalyst is selected from a group consisting of: dibutyl tin dilaurate, dibutyl tin diacetate, tetrabutyl titanate and tetraethyl titanate.

**27.** A desiccant matrix consisting essentially of:

30 to 80 matrix weight percent of a powdered molecular sieve desiccant in a carrier for said powdered molecular sieve desiccant, said carrier comprising an atmospheric curing resin which irreversibly partially crosslinks upon exposure to a component of an ambient atmosphere selected from the group consisting of oxygen and moisture, wherein said resin fully cures thereafter;

and

a polymerization catalyst.

**28.** The desiccant matrix of claim 27 wherein said catalyst is selected from a group consisting of: organotin compounds, amines and aliphatic titanates having from one to twelve carbon atoms.

**29.** A desiccant matrix consisting essentially of:

30 to 80 matrix weight percent of a powdered molecular sieve desiccant in a carrier for said powdered molecular sieve desiccant, said carrier comprising an atmospheric curing resin which irreversibly partially crosslinks upon exposure to a component of an ambient atmosphere selected from the group consisting of oxygen and moisture, wherein said resin fully cures thereafter;

and

an additive selected from a group consisting of: filler,

colorant, pigment and rheological agent.

**30.** The desiccant matrix of claim 29 wherein said plasticizer is selected from a group consisting of: phthalate ester, chlorinated paraffin, mineral oil and silicone oil.

**31.** A desiccant matrix consisting essentially of:

30 to 80 matrix weight percent of a powdered molecular sieve desiccant in a carrier for said powdered molecular sieve desiccant, said carrier comprising an atmospheric curing resin which irreversibly partially crosslinks upon exposure to a component of an ambient atmosphere selected from the group consisting of oxygen and moisture, wherein said resin fully cures thereafter;

and

a plasticizer.

**32.** The desiccant matrix of claim 31 wherein said plasticizer comprises greater than 0 and less than 30 matrix weight percent.

\* \* \* \* \*